

## UNITED STATES PATENT OFFICE

GEORGE HOLLAND ELLIS, HENRY CHARLES OLPIN, AND RALPH CHARLES STOREY, OF SPONDON, NEAR DERBY, ENGLAND, ASSIGNEES TO CELANESE CORPORATION OF AMERICA, A CORPORATION OF DELAWARE

## TREATMENT OF TEXTILE AND OTHER MATERIALS

No Drawing. Application filed June 7, 1930, Serial No. 459,828, and in Great Britain July 4, 1929.

This invention relates to the colouration by dyeing, printing, stencilling or otherwise of textile or other materials.

Vat colouring matters have long been employed on a very extensive scale for the colouration of cellulosic materials. The colouring matters have been applied to the said materials in the form of alkali salts of their reduction products, the so-called leuco compounds, and the colourations obtained have been highly valued on account of their resistance to the agencies to which textile materials are commonly subjected. The application of these vat colouring matters to other textile materials has in the past met with very serious difficulties owing either to the comparatively small affinity of the materials for the alkali salts of the leuco compounds, or to their being easily injured by the alkaline conditions existing in the dye vats. The application of the vat colouring matters to wool and silk, for instance, has in the past been principally confined to the use of a few colouring matters which can be vatted in the presence of small quantities of alkali.

The very remarkable discovery has been made that the free leuco compounds of vat colouring matters have good affinity for and can be directly applied to very many textile and other materials to produce valuable colourations thereon.

According to the present invention therefore, the colouration of textile or other materials made of or containing cellulose acetate or other organic derivatives of cellulose is effected by processes comprising the application of free leuco compounds of vat colouring matters. Vat colouring matters may thus be applied to the material in the absence of alkali, for example under neutral or acid conditions, a very great advantage in the treatment of cellulose ester materials. Moreover the affinities in relation to any particular fibre, of the leuco compounds of vat dyestuffs uncombined with alkalies in general differ considerably from those of the compounds of leuco bodies with alkalies. In consequence the invention renders possible the production of colourations, for example colourations on materials comprising two or more types of

fibre, which are difficult or impossible of attainment by hitherto known methods.

Free leuco compounds of the vat colouring matters may be applied to the textile or other materials in any convenient manner, for example in the form of solutions, e. g. in organic solvents. They are however most satisfactorily and conveniently applied in the form of aqueous dispersions or suspensions, and this method of application constitutes a very important feature of the present invention. Contrary to expectation, it has been found that the solutions, dispersions, or other preparations containing the free leuco compounds are remarkably stable in the presence of air.

Cellulose ester or ether materials show an exceptionally good affinity for the free leuco compounds, often greater than the affinity of the same materials for the alkali salts of the leuco compounds. For instance the free leuco compounds of the indigoid colouring matters have such remarkably good affinity for cellulose ester materials under neutral or acid conditions that it is even possible to rinse the materials before oxidizing the leuco compound, and colourations of excellent fastness to rubbing are thereupon obtained. In addition, as the dyeing operation can be effected under non-alkaline conditions, all danger of saponification of the cellulose ester may be avoided. A further valuable feature of the invention resides in the fact that the range of conditions for optimum dyeing is in general much wider than with alkaline vats. Thus, not only does the invention enable colouring to be effected under much less closely controlled conditions, but it much facilitates the application of mixtures of dyestuffs.

Vat dyestuffs of any desired kind may be employed for application according to the process of the present invention, and the term "vat dyestuff" is to be understood as comprising not only those colouring matters commonly employed for application to textile materials from alkaline vats, but any other colouring matters capable of yielding by reduction compounds which may be converted by oxidation into the original colouring matters. The following are given as in-

- stances of such colouring matters or classes of colouring matters:—
1. Indigo and allied colouring matters.
    - (a) Indigo and its derivatives, for example N.N'-dimethyl indigo and halogenated indigoes, e. g. Ciba blue 2B (Colour Index 1184).
    - (b) Halogenated indirubines, e. g. Ciba heliotrope B (Colour Index 1205).
    - (c) Thioindigo and its derivatives, for instance halogenated thioindigoid dyes, e. g. Ciba Bordeaux B (Colour Index 1208).
    - (d) Dinaphthindigoid dyes, e. g. Ciba green G (Colour Index 1198).
    - (e) Indigoid dyes obtainable by condensing isatins or thioisatins with  $\alpha$ -oxynaphthalenes or  $\alpha$ -oxy-anthracenes or derivatives thereof and if desired subsequently halogenating, e. g. Alizarin indigo 3R (Colour Index 1200) and Helindone blue 3GN (Colour Index 1203).
  2. Anthraquinone colouring matters.
    - (a) Simple amino-derivatives, e. g. 1-hydroxy-4-amino-anthraquinone; 1:5-diamino-4:8-dihydroxy-anthraquinone; 1-methylamino-anthraquinone; 1:4-dianilide-anthraquinone.
    - (b) Anthraquinone-quinolines, e. g. 1:2-dihydroxy-anthraquinone-quinoline (Colour Index 1066).
    - (c) Acylamino anthraquinones, e. g. 1-acetyl-amino-anthraquinone; 1:4-dipropionyl-aminoanthraquinone; 1:5-dibenzoylamino-anthraquinone (Colour Index 1132); succinyl-alphaamino anthraquinone (Colour Index 1139); 1:5-dibenzoylamino-4:8-dihydroxy-anthraquinone (Colour Index 1134).
    - (d) Anthrapyridones, e. g. 4-methylaminoanthrapyridone.
    - (e) Anthraquinone-mercaptans including their derivatives substituted in the nucleus and/or the mercapto groups.
    - (f) Benzanthonones and dibenzanthrones, e. g. Violanthrone (Colour Index 1099); Iso-violanthrone (Colour Index 1103); Amino-violanthrone (Colour Index 1102); Dimethoxy-dibenzanthrone (Colour Index 1101).
    - (g) Pyranthrone and its derivatives.
    - (h) Anthraflavone (Colour Index 1095).
    - (i) Anthraquinone acridones, e. g. anthraquinone 1(NH)-2(CO)-naphthacridone (Colour Index 1162).
    - (j) Dianthraquinonyls and acidylamino derivatives.
    - (k) Dianthraquinonylamines and derivatives, e. g. acidylamino derivatives.
    - (l) Anthraquinone azines and hydroazines, e. g. dianthraquinone-dihydroazines and their halogenated derivatives such as 1:2.1':2'-dianthraquinone azine (Colour Index 1106) and its dichlor derivatives (Colour Index 1113).
    - (m) Anthraquinone oxazines.
    - (n) Anthraquinone dioxides.
  - (o) Anthraquinone thiazines.
  - (p) Anthraquinone disulphides.
  - (q) Anthraquinone xanthones.
  - (r) Anthraquinone thioxanthones.
  - (s) Anthraquinone carbazoles.
  - (t) Anthraquinone thiiazoles.
  3. Derivatives of benzoquinone and naphthoquinones, e. g. those mentioned in United States patent applications S. Nos. 379,874 and 379,875 both filed 20th July, 1929.
  4. Indophenols and their derivatives, e. g. halogen derivatives.
  5. Perylene quinones and their amino, halogen and other derivatives.
  6. Dyestuffs obtainable by alkali fusion of imides and substituted imides of naphthalene peridicarboxylic acids and the dyestuffs obtainable by condensing naphthalene 1:4:5:-8-tetracarboxylic acids with mono- or diamines.
  7. Sulphur dyestuffs including not only those colouring matters commonly applied from sulphide baths but also those sulphur colouring matters commonly applied to cellulosic materials from hydrosulphite or other vats, for example the colouring matters obtained by sulphurizing indophenols derived from carbazol (see Colour Index Nos. 969, 970, 971, etc.)
  - Dispersions or suspensions of free leuco compounds of colouring matters may be obtained by any convenient means, whether mechanical or otherwise. For example the free leuco compounds themselves may be directly converted into aqueous dispersions by mechanical treatment or by treatment with dispersing agents and/or protective colloids. Alternatively the leuco compounds may be liberated or formed in the presence of dispersing agents and/or protective colloids, and in this manner dispersions or suspensions directly applicable for dyeing may be produced. For example vat colouring matters may be vatted with the aid of alkali and hydrosulphite or other reducing agents in the known manner and acidified with a suitable organic or inorganic acid in presence of protective colloids and/or dispersing agents. Moreover, the protective colloids or dispersing agents themselves may be converted by the acidification into other and even more suitable forms. The dispersing agents and protective colloids should be as stable as possible under the conditions in which the dispersions or suspensions are to be stored or applied. As examples of dispersing agents or protective colloids the following may be instanced:—
  - Sulphoaromatic fatty acid compounds, e. g. sulphobenzene palmitic acid compounds (see United States Patent No. 1,694,413).
  - Sulphoaromatic ricinoleic acid compounds, e. g. sulphonaphthalenericinoleic acid, (see United States patent application S. No. 134,138 filed 7th September, 1926).

Naphthenic acids or other carbocyclic compounds containing salt-forming groups or salts of such acids or compounds (see United States Patent No. 1,618,414).

5 Sulphonated oil compounds, e. g. sulphonated castor oil.

Furfural-naphthalene sulphonic acid compounds (see United States patent application S. No. 390,423 filed 4th September, 1929).

10 Resino-naphthalene sulphonic acid compounds (see United States patent application S. No. 390,424 filed 4th September, 1929).

Formaldehyde naphthalene sulphonic acid compounds.

15 Alkyl-, cycloalkyl-, and aralkyl-naphthalene sulphonic acids.

Sulphite cellulose waste liquor or its constituents or products of transformation, e. g. lignin sulphonic acid compounds.

20 Sulphonic acid compounds of mineral oils, tar oils, brown coal tar oils, and the like, and their products of condensation with alcohols.

Sulphonic acid compounds of distillation residues of benzaldehyde.

25 Molasses.

Carbohydrates including gums.

Glue and gelatine.

30 Aqueous dispersions or suspensions of the free leuco compounds may be acid, neutral or even slightly alkaline. For example they may have hydrogen ion concentrations corresponding to pH values lying between 3 and 9, for instance between 4 and 8. In general,

35 the colouration of cellulose acetate and other organic substitution derivatives of cellulose may be accomplished in a highly satisfactory

40 manner with aqueous suspensions or dispersions containing sufficient acetic, formic, or other organic acid to render them slightly acid to litmus.

The dispersions of the free leuco compounds may be prepared in the dyebaths themselves, or in the form of more or less concentrated liquid, paste, solid, or powdered

45 or other preparations which may be used for the preparation of dyebaths. Such preparations may be obtained for instance by removal of water by evaporation or otherwise from less concentrated dispersions, or by acidifying

50 concentrated solutions of alkali salts of leuco compounds of vat colouring matters in the presence of dispersing agents and/or protective colloids, or by simple grinding of the leuco compounds with dispersing agents

55 and/or protective colloids with or without water. The preparations preferably contain water and may receive additions of agents, e. g. reducing agents or acids, adapted to increase their stability in the presence of air.

60 These preparations comprise an important feature of the present invention, which further includes preparations which contain dispersing agents, particularly those referred to above, and/or protective colloids, together

65 with any compounds, e. g. the alkali salts of

the leuco bodies, from which the leuco compounds can be liberated or formed, for example by treatment with acids. The dispersing agent in the preparations containing either the free leuco bodies or compounds yielding them, will not necessarily be identical with that to be used in the dyebath, printing paste, etc., particularly as regards degree of acidity or alkalinity. The concentrated preparations may be employed for dyeing after dilution with water with or without addition of further quantities of protective colloids and/or dispersing agents, and after adjusting the acidity if necessary for the purpose in view.

70 The solutions or dispersions of free leuco compounds may be applied to textile or other materials in any convenient manner, for example by dyeing, padding printing, stenciling or the like. Aqueous dispersions or suspensions are preferably employed under neutral or acid conditions. If desired or requisite they may receive additions of thickening agents, for example when they are to be applied by padding or printing. Solutions or suspensions of free leuco compounds used according to the invention appear to be in general much more stable than the alkaline vats hitherto employed and in consequence manipulation of the materials is in many cases much facilitated. For example it is even possible to dye fabrics on winch machines or in open width on jigger machines, where in both cases there is a considerable passage of air through the material.

75 80 85 90 95 100 105 110 115 120 125 130

If desired the free leuco compounds of vat dyestuffs may be applied in conjunction with swelling agents for the materials to be coloured.

The oxidation of the leuco compounds on the materials may be effected by any suitable means, for example by simple air oxidation, treatment with bichromate and acid, treatment with bleaching powder, or treatment with soap and sodium perborate, and very satisfactory results have been obtained by oxidation in a bath containing soap and hydrogen peroxide, particularly as regards evenness of shade and little tendency of the resulting dyeings to rub.

The new process of colouration is applicable to any materials consisting of or containing cellulose esters or ethers and is particularly valuable in the colouration of such textile and other materials as are liable to injury by alkali, for example materials made of or containing cellulose esters, for example filaments, yarns, fabrics, ribbons and films made of these esters, e. g. cellulose acetate, formate, propionate, or butyrate, or the products obtained by the treatment of alkalinized cellulose with esterifying agents, for instance the product known as "immunized cotton" obtained with p-tolene sulpho chloride. The invention is also applicable to the colouration of

other organic substitution derivatives of cellulose for example cellulose ethers, e. g. methyl, ethyl, or benzyl cellulose, or the condensation products of cellulose and glycols or 5 other polyhydric alcohols. Particularly satisfactory colourations may for instance be produced on organic derivatives of cellulose in accordance with the invention by means of the free leuco compounds of indigoid and 10 thioindigoid colouring matters and colouring matters containing a single anthraquinone nucleus, for example of the following series:—anthraquinone acridones, oxazines, di-oxides, thiazines, disulphides, xanthones, 15 thioxanthones, carbazoles, and thiazoles. The importance of the invention will be appreciated in view of the low affinity or lack of affinity exhibited by cellulose acetate or other organic derivatives of cellulose for the alkali 20 compounds of leuco anthraquinone vat dyestuffs.

Mixed materials containing two or more kinds of textile fibres may be dyed by the process of the invention, the various fibres 25 being coloured in solid or contrasting shades according to their relative affinities for the colouring matter or matters; thus solid shades can be obtained on mixtures of cellulose acetate with wool or natural silk.

30 Cellulosic materials, for example cotton, linen, or the regenerated cellulose type of artificial silk show in general little or no affinity for the free leuco compounds of vat colouring matters applied in accordance with the 35 present invention. The new process therefore renders possible the production of valuable cross-dyed effects on certain mixed materials, for example on fabrics composed of 40 cellulose acetate and cotton, or natural silk and cotton, or cellulose acetate and a regenerated cellulosic type of artificial silk. For example the cellulose acetate in such a mixed material may be dyed with a dispersion of 45 the free leuco compound of a vat colouring matter, for example an indigoid or thioindigoid colouring matter or a colouring matter containing a single anthraquinone nucleus, so as to leave uncoloured the cotton or regenerated cellulose. The latter may then, if desired, be dyed with suitable colouring matters therefor. Alternatively the cellulosic portion of the material may be coloured prior to 50 the cellulose acetate part; for example the cellulosic portion may be dyed with a vat dyestuff in the presence of alkali salts of aromatic hydroxy compounds as described in U. S. Patent No. 1,716,720 so as to leave un- 55 stained the cellulose acetate and the latter then dyed with a vat dyestuff in the form of a dispersion of its free leuco compound.

The following examples show the best way known to us of carrying the invention into effect:—

### Example 1

200 grams of the brominated indigo known as Ciba blue G powder (Colour Index No. 1185) are pasted with 2.5 litres of the solution of sodium salt of sulphonaphthalene ricinoleic acid prepared according to Example A of U. S. Patent No. 1,694,413, and 40 to 50 litres of water at 60° C. added with stirring. 70 200 grams of caustic soda are now added, and 350 grams of sodium hydrosulphite sprinkled in with good stirring, and stirring continued for 5–10 minutes or till reduction is complete, after which the liquor is filtered into a dyebath containing 500 litres of soft 75 water at 50° C. to which 50 grams of hydrosulphite have previously been added. The dyebath is now rendered slightly acid to litmus by careful addition of approximately 3 litres of 10% acetic acid, whereby the free 80 leuco compound is obtained as a very satisfactory dispersion. 10 kilograms of cellulose acetate yarn in hank form are now entered, and the temperature raised to 75–80° C. in 1/2 hour and held thereabouts for 1/2 to 3/4 85 hour.

The goods are now lifted, rinsed in soft water, hydro-extracted, and hung up to oxidize, after which they are given a light soaping in a 1 gram per litre soap bath to which 90 perborate may advantageously be added, rinsed, and dried or otherwise treated as requisite.

### Example 2

200 grams of the vat dyestuff known as 100 Caledon jade green (Colour Index No. 1101) are pasted with 2.5 litres of a highly sulphonated castor oil stable to dilute organic acids, suitably diluted, and vatted with 200 grams of caustic soda and 350 grams hydrosulphite as in Example 1. The clear solution is now added to the dyebath previously set with hydrosulphite, acidified, and 10 kilos of cellulose acetate yarn in hank form entered and processed exactly as detailed in that example. 105 After oxidation, and soaping, the goods which are now dyed a bright green shade, are rinsed and dried or otherwise treated as requisite.

In the same manner cellulose acetate yarns may be coloured in red shades by means of Caledon red BN (Colour Index 1162), or in yellow shades by means of 2':5'-dichloro-1:2-anthraquinone thioxanthone.

### Example 3

200 grams of the indophenol dyestuff prepared by oxidation of p-aminodimethylaniline and alphanaphthol (Colour Index No. 831) are pasted with 1 litre of sulphite cellulose liquor, or an equivalent quantity of a suitable product of transformation, and 40 to 50 litres of water at 60° C. are added with stirring. 200 grams of caustic soda are now added and 300 grams hydrosulphite sprinkled in with stirring, and stirring con- 120 125 130

tinued till vatting is complete, after which the liquor is filtered into a suitable dyebath containing 500 litres of soft water at 50° C. previously set with 50 grams of hydrosulphite. The dyebath is now acidified by careful addition of approximately 3 litres of 10% acetic acid, and 10 kilograms of cellulose acetate woven fabric entered, after which the temperature is raised to 75 to 80° C. in 1/2 hour and held thereabouts for 1/2-3/4 hour.

10 The goods are now lifted, rinsed, hydroextracted, and allowed to oxidize in the air, or in a bath containing 1 gram per litre soap and 2 grams per litre sodium perborate till 15 the colour is fully developed, after which they are lifted, rinsed, and dried or otherwise treated as requisite.

*Example 4*

20 1 kilogram of a well ground 20% aqueous paste of the leuco compound of 1 benzoyl-amino-4-oxy-anthraquinone is added to a solution of 150 grams of gelatine dissolved in 25 10 litres of water rendered faintly acidic with acetic acid. The whole is warmed to 80° C. and stirred to ensure efficient dispersion, and then diluted in a suitable machine to 300 litres with warm soft water. 30 10 kilos of a woven fabric consisting of equal parts of wool and cellulose acetate previously well wetted out, are now entered, and dyeing carried out 1/2 hour to 75-80° C. and 3/4 hour at 75° C. or thereabouts. The goods 35 are now lifted, rinsed, and oxidized by treating for 5 minutes at 60° C. in a 300 litre bath containing 50 grams bichromate of soda, and 250 ccs. 10% sulphuric acid.

40 The goods are now lifted, rinsed, soaped lightly, washed off well, and dried or otherwise treated as requisite. Both fibres are dyed in full shades of pink.

*Example 5*

45 To dye 10 kilos of a woven fabric consisting of equal parts of cotton and cellulose acetate, the cotton green and the cellulose acetate orange:—

50 The cotton is first dyed with 2% of its weight of Caledon jade green (Colour Index No. 1101) from a sodium phenate-hydrosulphite vat according to the methods detailed in U. S. Patent No. 1,716,720.

55 The cellulose acetate portion is now dyed as follows:—

60 1500 grams of a 10% paste of the leuco compound of 1-amino-2-methyl-anthraquinone are stirred with 500 ccs. of neutral or very faintly acid Turkey red oil (50%). 65 The whole is heated to 95° C. with stirring, and stirred till a good dispersion is achieved. The whole is now diluted suitably with hot soft water and added through a filter cloth to a dyebath containing 300 litres of soft water from which dissolved oxygen has been

removed by addition of the requisite quantity of hydrosulphite. The goods are now entered, and the temperature raised to 75° C. in 3/4 hour and held thereabouts a further 70 3/4 hour. They are now lifted, rinsed, and treated 75 3/4 hour at 60° C. in a bath containing 1 gram per litre soap and 2 grams per litre sodium perborate. The goods are now lifted, rinsed and dried or otherwise treated as requisite.

*Example 6*

Cellulose acetate woven fabric previously dyed with a violet dyestuff dischargeable with formosul, for example the dyestuff obtained by coupling diazotized 3:5-dinitro-2-amino-anisole with alphanaphthylamine, is printed with a printing paste prepared as follows:—

|                                                                                  | Grams | 85 |
|----------------------------------------------------------------------------------|-------|----|
| Gum arabic 1:1                                                                   | 560   |    |
| Ciba pink B                                                                      | 30    |    |
| Sodium sulpho-naphthalenericinoleate prepared as in U. S. Patent No. 1,694,413   | 50    | 90 |
| Caustic soda                                                                     | 30    |    |
| Water                                                                            | 140   |    |
| Hydrosulphite                                                                    | 40    |    |
| The above are heated till vatted, cooled, and a liquor consisting of a mixtue of |       |    |
|                                                                                  | 95    |    |
| Formic acid 40%                                                                  | 90    |    |
| Formosul                                                                         | 60    |    |

added slowly with good stirring. The amount of liquor added should be just sufficient to neutralize or render the paste only faintly acid. After printing the goods are dried, passed through a rapid ager or other suitable steaming device, and then oxidized at 60° C. for 5 minutes in a bath containing 100 2.5 grams per litre chrome and 5 grams per litre sulphuric acid. The goods are now rinsed, soaped well, washed off, and dried or otherwise treated as requisite.

What we claim and desire to secure by 110 Letters Patent is:—

1. Process for the coloration of textile and other materials containing organic derivatives of cellulose comprising applying thereto free leuco compounds of vat dyestuffs. 115

2. Process for the coloration of textile and other materials containing organic derivatives of cellulose comprising applying thereto free leuco compounds of vat dyestuffs in the form of aqueous dispersions. 120

3. Process for the coloration of textile and other materials containing organic derivatives of cellulose comprising applying thereto free leuco compounds of vat dyestuffs in the form of aqueous dispersions having a pH 125 value between 3 and 9.

4. Process for the coloration of textile and other materials containing organic derivatives of cellulose comprising applying thereto free leuco compounds of vat dyestuffs in 130

- the form of aqueous dispersions having a slightly acid reaction.
5. Process for the coloration of textile and other materials containing organic derivatives of cellulose comprising applying thereto a composition comprising a free leuco compound of a vat dyestuff and a dispersing agent.
6. Process for the coloration of textile and other materials containing cellulose acetate comprising applying thereto free leuco compounds of vat dyestuffs.
7. Process for the coloration of textile and other materials containing cellulose acetate comprising applying thereto free leuco compounds of vat dyestuffs in the form of aqueous dispersions.
8. Process for the coloration of textile and other materials containing cellulose acetate comprising applying thereto free leuco compounds of vat dyestuffs in the form of aqueous dispersions having a pH value between 3 and 9.
9. Process for the coloration of textile and other materials containing cellulose acetate comprising applying thereto free leuco compounds of vat dyestuffs in the form of aqueous dispersions having a slightly acid reaction.
10. Process for the coloration of textile and other materials containing cellulose acetate comprising applying thereto a composition comprising a free leuco compound of a vat dyestuff and a dispersing agent.
11. Process for the coloration of textile and other materials containing organic derivatives of cellulose comprising applying thereto free leuco compounds of indigoid vat dyestuffs.
12. Process for the coloration of textile and other materials containing cellulose acetate comprising applying thereto free leuco compounds of indigoid vat dyestuffs.
13. Process for the coloration of textile and other materials containing cellulose acetate comprising applying thereto a composition comprising a free leuco compound of an indigoid vat dyestuff and a dispersing agent.
14. Process for the coloration of textile and other materials containing organic derivatives of cellulose comprising applying thereto free leuco compounds of anthraquinone vat dyestuffs.
15. Process for the coloration of textile and other materials containing cellulose acetate comprising applying thereto free leuco compounds of anthraquinone vat dyestuffs.
16. Process for the coloration of textile and other materials containing organic derivatives of cellulose comprising applying thereto free leuco compounds of anthraquinone vat dyestuffs containing only one anthraquinone residue.
17. Process for the coloration of textile and other materials containing cellulose acetate comprising applying thereto free leuco compounds of anthraquinone vat dyestuffs containing only one anthraquinone residue.
18. Process for the coloration of textile and other materials containing cellulose acetate comprising applying thereto a composition comprising a free leuco compound of an anthraquinone vat dyestuff containing only one anthraquinone residue and a dispersing agent.
19. Process for the coloration of textile and other materials containing cellulose acetate comprising applying thereto free leuco compounds of aminoanthraquinones.
20. Process for the coloration of textile and other materials containing organic derivatives of cellulose comprising applying thereto a preparation made by vatting a vat dyestuff in alkaline medium and adding in the presence of a dispersing agent at least sufficient acid to separate free leuco compound of the dyestuff.
21. Process for the coloration of textile and other materials containing cellulose acetate comprising applying thereto a preparation made by vatting a vat dyestuff in alkaline medium and adding in the presence of a dispersing agent at least sufficient acid to separate free leuco compound of the dyestuff.
22. Process for the coloration of textile and other materials containing organic derivatives of cellulose and animal fibres comprising applying thereto free leuco compounds of vat dyestuffs.
23. Process for the coloration of textile and other materials containing cellulose acetate and animal fibres comprising applying thereto free leuco compounds of vat dyestuffs.
- In testimony whereof we have hereunto subscribed our names.
- GEORGE HOLLAND ELLIS.  
HENRY CHARLES OLPIN.  
RALPH CHARLES STOREY.

**CERTIFICATE OF CORRECTION.**

Patent No. 1,900,172.

March 7, 1933.

**GEORGE HOLLAND ELLIS, ET AL.**

It is hereby certified that error appears in the printed specification of the above numbered patent requiring correction as follows: Page 1, line 55, after "materials" insert the words "made of or containing cellulose acetate or other organic derivatives of cellulose"; and that the said Letters Patent should be read with this correction therein that the same may conform to the record of the case in the Patent Office.

Signed and sealed this 9th day of May, A. D. 1933.

**M. J. Moore.**

(Seal)

**Acting Commisioner of Patents.**